

## UNITED STATES PATENT OFFICE

2,289,258

## PROCESS FOR THE MANUFACTURE OF IRON OXIDE

Thomas Glenwright French, Newcastle-on-Tyne, England, assignor to The Priestman Collieries Limited, Newcastle-on-Tyne, England, a British company

No Drawing. Application October 16, 1939, Serial No. 299,761. In Great Britain September 30, 1938

3 Claims. (Cl. 23—200)

This invention relates to processes for the manufacture of iron oxide of the kind comprising precipitating a ferrous hydroxide by the electrolysis with iron electrodes of a solution of ionizable alkaline metal salts such as sodium and/or potassium salt.

The object of the invention is to provide a process for the manufacture of iron oxide for use mainly as a black, brown or red pigment of maximum purity, and which will be cheaper to carry into effect than has been the case hitherto.

Heretofore proposals have been made for the production of iron oxide for the manufacture of pigments which have consisted in precipitating a ferrous oxide by the chemical process of adding hydrate of lime, carbonate of soda or the equivalent, to a solution of a ferrous salt such as ferrous sulphate, and oxidising the precipitated ferrous oxide by blowing air into the solution containing the precipitate to convert the ferrous to ferric oxide. In another proposal, the ferrous oxide was precipitated electrolytically, removed from the electrolytic bath, washed and dried, and then roasted to produce ferric oxide. According to another electrolytic process, the solutions produced at the respective electrodes were each led away in separate streams and subsequently brought together outside the electrolysis cell to precipitate the ferrous oxide which was subsequently oxidised in its mother liquor.

I have found that by producing the iron oxide electrolytically, a finer quality of pigment is obtained than with chemical methods, and according to the present invention the electrolytic precipitation of the ferrous hydroxide is combined with the step of oxidising the ferrous oxide precipitated while still in suspension in the electrolytic bath to produce a ferric-ferrous hydroxide.

In addition to the improved quality of pigment obtained by electrolytic precipitation of the iron oxide as above mentioned, the process according to the invention reduces the number of reagents employed to a minimum, and, with the convenience of cheap electric power for the electrolytic precipitation, enables the complete process to be carried out in one industrial—as distinct from chemical—operation, and so gives an improved product by means of a cheap and convenient process.

In order to obtain maximum purity the electrolysis current is preferably reversed at intervals of about 30 minutes. Otherwise there is a tendency for metallic iron coming down as black specks.

According to one process an electrolyte of sodium chloride or sodium sulphate of density sp. gr. 1.10 is introduced into wood vats, into which are placed iron or mild steel anodes connected to a supply of D. C. current.

The electrolyte is maintained at a temperature of 80° to 90° C., and the current density is approximately .3 amp. per square inch.

The electrolysis produces a bluish white precipitate of ferrous hydroxide of an extremely tenuous nature. Owing to the exposure of the electrolyte to the atmosphere, this precipitate in time would become oxidised to a black ferric-ferrous hydroxide. However to accelerate the process of oxidation, air is continuously blown into the electrolyte. The continuous blowing of air into the electrolyte also results in a precipitate which settles easily and more readily separates from the electrolyte by filtration in a filter press. The black hydroxide is washed with water in a filter press, dried in a hot air oven at 100° C., and subsequently ground to the requisite fineness in a suitable mill.

The product after drying is a black hydroxide of iron, stable at 100° C.

To produce other colours of oxide from brown to deep red, the black hydroxide is calcined in a suitable furnace with excess air, the degree of temperature affecting the resulting colour. For example, at 200° C. a brown pigment is obtained, at 600° C. a bright Turkey red is obtained, at 800° C. a deep Turkey red and at 1000° C. an Indian red pigment is produced.

In order to produce a maroon or ochre like pigment, in an alternative process the paste from the filter press is mixed with water to form a slurry. To the slurry is added an oxidizing agent, preferably a solution of sodium hypochlorite, which oxidizing agent is preferably made by electrolysis of sodium chloride. The whole mixture is then boiled until a ferric hydroxide of uniform light brown colour is obtained. Ferrous sulphate is then added and the boiling continued until a ferric hydroxide ochre pigment known as ferrite yellow is formed.

The pigment is separated by means of a filter press, washed with water and the paste dried in an air oven.

If desired air may be blown through in addition to the step of adding the oxidizing agent. It is important that the oxidizing agent be introduced apart from the electrolyte.

By calcining with excess of air as mentioned in connection with the first process a similar

range of shades from light maroon or ochre to dark maroon may be obtained.

According to one example of the above alternative process, an electrolysis vat containing sodium chloride is connected in closed circuit with the mixing vat. Sodium hypochlorite from the electrolysis vat is admitted to the mixing vat and at the same time the mixture in the mixing vat is subjected to boiling. Sodium hypochlorite is continued to be admitted to the mixing vat until the required amount of oxidation has taken place as a result of the combined action of the sodium hypochlorite and the boiling. When this stage is reached, the resulting brown ferric hydroxide is allowed to settle in the mixing vat.

In this reaction the sodium hypochlorite has given up its oxygen and has been converted back to the original sodium chloride which is available for fresh electrolysis. Virtually therefore the sodium chloride acts as a convenient oxygen carrier, the electrolysis supplying the oxygen. This process yields the further economic advantage that the same substance serves for the two electrolysis processes.

After the ferric hydroxide has settled, the liquor in the mixing vat—which is sodium chloride—is pumped back to the electrolysis vat.

Ferric sulphate is now added to the paste in the mixing vat and boiling is continued until the ferric hydroxide ochre or ferrite pigment is obtained.

The pigment is then transferred to a second filter press, separated and washed and dried, and if desired calcined to temperatures depending on the depth of colour required.

By the process according to the invention iron oxide pigment from black to deep reds, maroons or ochres of a purity of 99.5% is obtained.

I claim:

1. The process for producing maroon or ochre like pigments, comprising precipitating ferrous hydroxide by the electrolysis with iron electrodes of a solution of an ionizable alkali metal salt, and oxidising the ferrous hydroxide precipitated while in suspension in the electrolysis bath to produce a ferric ferrous hydroxide, washing with

water the ferric ferrous hydroxide, separating the said hydroxide, mixing the hydroxide with water to form a slurry, adding an oxidising agent to said slurry, boiling the mixture until a ferric hydroxide of uniform light brown colour is obtained, then adding ferrous sulphate and continuing boiling until a ferric hydroxide ochre pigment known as ferrite is obtained.

2. The process for producing maroon or ochre like pigments, comprising precipitating ferrous hydroxide by the electrolysis with iron electrodes of a solution of an ionizable alkali metal salt, and oxidising the ferrous hydroxide precipitated while in suspension in the electrolysis bath to produce a ferric ferrous hydroxide, washing with water the ferric ferrous hydroxide, separating the said hydroxide, mixing the hydroxide with water to form a slurry, adding sodium hypochlorite to said slurry, boiling the mixture until a uniform light brown colour is obtained, then adding ferrous sulphate and continuing boiling until a ferric hydroxide ochre pigment known as ferrite is obtained.

3. The process for producing maroon or ochre like pigments, comprising precipitating ferrous hydroxide by the electrolysis with iron electrodes of a solution of an ionizable alkali metal salt, and oxidising the ferrous hydroxide precipitated while in suspension in the electrolysis bath to produce a ferric ferrous hydroxide, washing with water the ferric ferrous hydroxide, separating the said hydroxide, mixing the hydroxide with water to form a slurry, adding to said slurry sodium hypochlorite which is obtained by the electrolysis of sodium chloride, the sodium hypochlorite giving up its oxygen during the first boiling and the resulting restored sodium chloride being used again in the electrolysis process for producing the sodium hypochlorite, the same sodium chloride thus being usable continually as an oxygen carrier for the oxidation step, boiling the mixture until a uniform light brown colour is obtained, then adding ferrous sulphate and continuing boiling until a ferric hydroxide ochre pigment known as ferrite is obtained.

THOMAS GLENWRIGHT FRENCH.